

## UNITED STATES PATENT OFFICE.

CHARLES T. EVANS, OF TITUSVILLE, PENNSYLVANIA, ASSIGNOR TO CYCLOPS STEEL COMPANY, OF NEW YORK, N. Y., A CORPORATION OF NEW YORK.

## ALLOY.

No Drawing. Application filed October 3, 1919, Serial No. 328,336. Renewed August 8, 1924.

*To all whom it may concern:*

Be it known that I, CHARLES T. EVANS, a citizen of the United States, residing at Titusville, county of Crawford, and State of Pennsylvania, have invented certain new and useful Improvements in Alloys, fully described and represented in the following specification.

This invention relates to a new alloy having the characteristics of steel, which is non-corrosive, and which possesses the highly desirable qualities of hardness and toughness, so that it is fitted for the manufacture of articles of various kinds in which a non-corrosive steel is desirable.

The non-corrosive, or so-called "stainless" steels now on the market are usually made by adding chromium in considerable quantities to iron, that is, in percentages from 9% to 16%, these steels differing in this respect from the so-called high speed steels which contain a lower percentage of chromium. These so-called "stainless" steels do not develop the non-corrosive characteristic until after working, that is, until after the subsequent heat treatment and sometimes not until after polishing.

It follows, therefore, that articles made from it may not be entirely non-corrosive. In making table cutlery, for instance, the blades which are tempered and polished may be non-corrosive, whereas the tang or shank and the collar which separates the tang from the blade, not being subjected to this treatment, do not exhibit the same non-corrosive characteristic as the blade. Further, the high chromium content of the alloy renders it brittle, so that the cost of working the material is high and is attended by considerable loss, thus rendering the steel unduly expensive.

It is the object of this invention to produce an alloy having the characteristics of steel, which is non-corrosive, that is, an alloy which is not attacked by vegetable acids nor corroded by the action of the atmosphere, and in which the alloy itself has this quality, that is, neither subsequent heat treatment nor polishing are necessary to develop the non-corrosive characteristic.

In common with all other steels, the basis of this novel steel is iron. By the term "iron", it will be understood that an iron which has a low carbon content and which has been through the usual refining pro-

cesses is meant. Pig iron, for instance, which contains a large percentage of impurities, such, for instance, as sulphur and phosphorous, is not suitable for the purpose. In other words, the iron must have gone through the usual refining processes for the purpose of eliminating the impurities.

Unless the iron employed contains a considerable percentage of silicon, silicon is added to it, and there is also added at least one other refractory metal of the carbon group. A refractory metal of the carbon group which gives excellent results is zirconium. The percentage of silicon and zirconium, if this member of the carbon group be added, may vary within wide limits, it being understood that when the percentage of silicon is high, less zirconium need be added than when the percentage of silicon is low, and vice versa. Fairly good results have been obtained from an alloy of iron, zirconium and silicon where the combined percentage of silicon and zirconium in the alloy is 2.6%, the zirconium in this mixture being as low as .1%. Better results will be obtained, however, if the silicon content be lowered somewhat and the zirconium content increased. Excellent results have been obtained from an alloy in which the percentage of zirconium was about 1%, the percentage of silicon in this instance being also about 1%.

If a harder steel be desired than that produced by the combination of iron, silicon and zirconium, a hardening material may be added. Chromium, for instance, may be added to the alloy. The addition of chromium hardens and toughens the alloy, but this metal also increases its refractory character, and, therefore, makes the alloy brittle, and, consequently, renders it more difficult to work economically. Where, a hardening metal, such as chromium is added, it is, therefore, desirable to add metals to the alloy which will modify this refractory characteristic. This may be accomplished by adding nickel and also manganese. Excellent results have been obtained by thus adding nickel and manganese to an alloy containing iron, silicon, zirconium and chromium. The nickel and manganese render the alloy more malleable and ductile, so that it can be more economically worked, and they also improve the non-corrosive

60

65

70

75

80

85

90

95

100

105

110

qualities. When any or all of these metals are added, the percentage or percentages may be considerably varied. Excellent results have been obtained by the addition of 5 about 7% chromium, about 19% nickel, and about 2.5% manganese, though it is to be understood that these percentages are illustrative merely. For instance, good results have been obtained where the percentage of 10 chromium is as low as 3%. It may also be remarked that less silicon and zirconium are necessary when chromium, nickel and manganese are used in the alloy. A small addition of copper to the alloy, say, about .3%, 15 will also add to the non-corrosive quality of the alloy.

The alloy or steel above described is non-corrosive in the ingot, and any article made therefrom is non-corrosive throughout. 20 Further, the material is highly ductile and malleable, so that it can be readily worked with comparatively small losses, and it is, therefore, well adapted to a wide range of uses.

25 What is claimed is:

1. An alloy having the characteristics of steel and comprising iron, and silicon and zirconium, the combined percentage of silicon and zirconium being not less than 2% 30 nor more than about 2.6%.
2. An alloy having the characteristics of steel and comprising iron, silicon and zirconium and chromium, the combined per-

centage of silicon and zirconium being about 2%. 35

3. An alloy having the characteristics of steel and comprising iron, silicon, zirconium and chromium, the combined percentage of silicon and zirconium being about 2% and the chromium percentage being from about 40 3% to about 7%.

4. An alloy having the characteristics of steel and comprising iron, silicon, zirconium, chromium and manganese, the combined percentage of silicon and zirconium being about 2%, and the chromium from about 45 3% to about 7%.

5. An alloy having the characteristics of steel and comprising iron, silicon, zirconium, chromium, nickel and manganese, the combined percentage of silicon and zirconium being about 2%, the chromium from about 50 3% to about 7%, and the nickel from about 5% to about 20%.

6. An alloy having the characteristics of steel and comprising iron, silicon, zirconium, chromium, nickel and manganese, the percentages being such that the resultant alloy 55 is resistant to corrosive influences and is hard and tough, and a small percentage of copper, whereby the non-corrosive quality 60 of the alloy is increased.

In testimony whereof, I have hereunto set my hand.

CHARLES T. EVANS.